

Aug. 25, 1959

L. SAIVES

2,901,384

METHOD FOR TREATING CAST IRON CASTINGS

Filed Feb. 10, 1953

Fig.1



Fig.2



Fig.3



# United States Patent Office

2,901,384

Patented Aug. 25, 1959

1

2,901,384

## METHOD FOR TREATING CAST IRON CASTINGS

Leon Saives, Billancourt, France, assignor to Regie Nationale des Usines Renault, Billancourt, France

Application February 10, 1953, Serial No. 336,187

Claims priority, application France February 20, 1952

9 Claims. (Cl. 148—3)

The invention relates to a method of treating white 15 cast iron with a view to increasing its toughness.

It is known that copper and nickel facilitate the graphitisation of castings both during the solidification of grey cast iron and during the annealing of white cast iron which can be rendered malleable. It is likewise 20 accepted that nickel is more effective than copper and it is current practice to put up to 5% nickel in high quality grey cast iron but it is not customary to introduce copper or nickel into white cast iron which can be rendered malleable with a black heart, the effect of 25 these constituents not being sufficient to compensate for the increase in price.

This invention is characterised by the fact that in white cast iron which can be rendered malleable, the copper, which is present in a concentration of 0.7% 30 to 3%, may have an effectiveness which is very great and quite unexpected, if the graphitisation treatment is carried out in three successive phases:

(1) Austenisation above the temperature for the end of the eutectoid transformation followed by chilling in 35 stages;

(2) Tempering of and formation of nuclei in the graphite by sudden re-heating or better still by progressive heating to a precise suitable temperature T, of the order of 450° C., viz. lying between 400° C. and 500° C., and lasting a sufficient length of time, e.g. 24 to 100 40 hours, more particularly for a period of the order of 36 to 48 hours. In metal chill molds, tempering is suitably carried out for 1 to 24 hours.

(3) Graphitisation of the primary cementite by prolonged maintenance at a temperature considerably higher than the temperature for the end of the eutectoid transformation, e.g. 875° C. to 900° C. for a period of time sufficient for the total disappearance of the cementite, more particularly 12 hours at 895° C. or 3 hours at 900° C. followed, for example, by cooling in still air. Graphitization may also be carried out, for example, at 875 to 895° C. for one-half to two hours.

In order to demonstrate this new property of copper, examples are given to show that the action of copper is more effective than that of an equal quantity of nickel; bearing in mind the fact that nickel is about five times more expensive than copper, the effectiveness for the same cost of addition is of a much higher order and offers a considerable industrial advantage.

It is possible to ascertain the comparative action of the constituents copper and nickel by working on eutectoid steels with a composition similar to that of white cast iron, that is to say, the composition of which is obtained by deduction from the primary cementite or proeutectoid.

Four steels were cast, then austenised at 810° C. 30 minutes, oil-hardened, reheated for 48 hours at T°, cooled in still air, reheated to 700° C. for 150 hours and then cooled in still air. The average number N of 70 granules of graphite formed per mm.<sup>2</sup> section is given below, beside the chemical compositions, and for two

2

values of T. For the optimum value of T=450° C., nickel does not bring any improvement in comparison with other cast steels of the same composition, whereas copper, on the other hand, increases the number of nuclei per unit of section by 5,000.

| Castings | C    | Si   | Mn   | Ni   | Cu   | T=450° C.          | T=500° C.          |
|----------|------|------|------|------|------|--------------------|--------------------|
|          |      |      |      |      |      | N/mm. <sup>2</sup> | N/mm. <sup>2</sup> |
| 1.893    | 0.96 | 1.27 | 0.34 | 0    | 0    | 30,000             | 3,000              |
| 2.064    | 0.92 | 1.55 | 0.39 | 0.64 | 0    | 30,000             | 10,000             |
| 2.067    | 0.93 | 1.51 | 0.35 | 0    | 1.60 | 35,000             | 16,000             |
| 2.063    | 0.95 | 1.70 | 0.40 | 0.58 | 1.68 | 35,000             | 16,000             |

Passing now to the comparison of white cast iron which can be rendered malleable, it will be seen that the castings appearing in the following table were cast in sand in bars of 15 x 30 mm. and produced a white structure. They were then subjected to the following series of treatments: austenisation at 810° C. lasting 30 minutes, quenching in a salt bath at 180° C. for 1 minute, cooling in still air, reheating to T=450° C. for 48 hours, cooling in still air, reheating to 885° C. for 10 hours and cooling in still air. In each case, the graphitisation of the primary cementite is complete. The chemical compositions and the average number N of grains of graphite (fine nodules or ultra fine spherules as the case may be) per mm.<sup>2</sup> are given in the following table:

| Castings | C    | Si   | Mn   | Cu   | Ni   | S     | P     | N     |
|----------|------|------|------|------|------|-------|-------|-------|
| 2.050    | 2.40 | 1.02 | 0.40 | 0    | 2.08 | 0.108 | 0.094 | 2,500 |
| 2.045    | 2.39 | 1.08 | 0.38 | 0    | 2.13 | 0.094 | 0.097 | 2,500 |
| 2.041    | 2.28 | 1.43 | 0.66 | 2.00 | 0    | 0.10  | 0.09  | 9,000 |
| 2.040    | 2.32 | 1.08 | 0.40 | 2.02 | 0    | 0.107 | 0.094 | 9,500 |

It will be seen that with an equal concentration, copper produces more than 3.7 to 4 times the number of nodules of graphite. Assuming that nickel is 5 times more expensive than copper, the effectiveness of copper is about twenty times greater than that of nickel for the same price of addition.

If a comparison is now made with castings devoid of nickel and copper, cast under the same conditions as above and with the same preliminary hardening and nuclear formation treatment as above, but the graphitisation being for 14 hours at 895° C., the slight coalescence of the nodules of graphites has slightly diminished their number. The number of nodules N per sectional unit and the percentage of residual cementite Fe<sub>3</sub>C found are indicated in the following table:

| Castings | C    | Si   | Mn   | Cu  | Ni   | S    | P     | N     | Fe <sub>3</sub> C |
|----------|------|------|------|-----|------|------|-------|-------|-------------------|
| 2.145-1  | 2.32 | 1.46 | 0.67 | 0   | —    | 0.11 | 0.095 | 2,500 | —                 |
| 2.145-11 | 2.22 | 1.42 | 0.66 | 0   | 1.83 | 0.10 | 0.095 | 2,770 | 0.5               |
| 2.147    | 2.33 | 1.53 | 0.71 | 2.2 | 0.1  | 0    | 0.12  | 6,550 | 0                 |

The increase in the number of nodules or spherules of graphite is 12.3 times greater in the case of copper than in that of nickel, given the same quantity of addition. Bearing in mind the fact that nickel is five times more expensive than copper, the effectiveness, for the same cost of addition, is sixty times greater in the case of copper.

If the comparison is made, but with a slightly different treatment, the same preliminary hardening, nuclear formation for 48 hours at T=500° C. graphitisation for 10 hours at 885° C., the following results are obtained:

| Castings | C    | Si   | Mn   | Cu   | Ni   | S     | P     | N     |
|----------|------|------|------|------|------|-------|-------|-------|
| 1.995    | 2.36 | 1.15 | 0.36 | 0    | 0    | 0.12  | 0.10  | 1,000 |
| 2.045    | 2.39 | 1.08 | 0.38 | 0    | 2.13 | 0.094 | 0.097 | 1,350 |
| 2.041    | 2.28 | 1.43 | 0.66 | 2.00 | 0    | 0.10  | 0.09  | 6,900 |

The increase in the number of nodules, given the same concentration of addition is 18 times greater for copper than for nickel. Price for price, the effectiveness of the copper is 90 times greater than that of nickel.

It is known that in malleable castings without special additions, the preliminary hardening must of necessity be martensitic, which is what has been done in the examples given above; but another remarkable property of copper has been discovered, namely that it enables a large number of fine nodules to be obtained by means of a preliminary bath-hardening. After the preliminary bath-hardening carried out, the nuclear formation of the graphite is obtained by annealing for 48 hours at 450° C. and the graphitisation is then obtained by reheating to 895° C. and maintaining at this temperature for 14 hours, followed by cooling in still air. Between the cycles in this treatment, there is a return to room temperature, but it goes without saying that the passage from 400° C. to 450° C. then to 895° C. could be made without any intermediate cooling and with the same re-

producing very fine and very diffuse graphite, which, however, because of its stability, develops at the expense of the primary cementite in the subsequent high temperature operation. Nickel, on the other hand, because of its high solubility in ferrite, has an average composition throughout and its effectiveness remains low.

In these treatments of casting containing copper, an essential characteristic is to observe, the succession of the three operations: preliminary hardening, nuclear formation towards 450° C., subsequent graphitisation at a high temperature.

An example is given by comparing the correct procedure and two other procedures in which either the preliminary hardening or the tempering for nuclear formation has been omitted. In this experiment, the control casting without copper is the casting 1995 already mentioned; the analysis of casting 1996 is C=2.45%; Si=1.14%; Mn=0.48%; S=0.12%; P=0.10%; Cu=2.00%.

20 The results are given in the following table:

|                       | Series of treatments  |                             |                        | Residual, Fe <sub>3</sub> C% |            | N             |            |
|-----------------------|-----------------------|-----------------------------|------------------------|------------------------------|------------|---------------|------------|
|                       | Preliminary hardening | Tempering Nuclear formation | Primary graphitisation | Control, 1995                | Cu=2% 1996 | Control, 1995 | Cu=2% 1996 |
| Nil                   | 450°, 48 h.           | 875°, 10 h.                 |                        | 18                           | 5          | 0             | 80         |
| 810° C., 30 min. Salt | Nil                   | 875°, 10 h.                 |                        | 15                           | 1          | 110           | 300        |
| 180° C., 1 minute.    |                       |                             |                        |                              |            |               |            |
| 810° C., 30 min. Salt | 450°, 48 h.           | 875°, 10 h.                 |                        | 5                            | 0          | 200           | 6,500      |
| 180° C., 1 minute.    |                       |                             |                        |                              |            |               |            |

sult. At the same time, it was desired to demonstrate this remarkable property of copper in causing the preliminary hardening at the actual temperature of the nuclear formation of the graphite: for this purpose, the castings were austenised at 810° C. for 30 minutes, hardened at 450° C. and maintained for 48 hours at this temperature, then heated to 895° C. for 14 hours and then cooled in still air.

For these two series of treatments, and for castings of the compositions already given (always cast in sand in bars 15 x 30 mm., the structure of the casting being perfectly white), the following table gives the results in relation to the percentage of residual primary cementite Fe<sub>3</sub>C and the number N of nodules or spherules of graphite per mm.<sup>2</sup> of section.

35 It will be seen that only the triple treatment and the addition of copper make it possible to reabsorb the entire quantity of primary cementite and to have a large number of nodules or spherules of graphite.

40 In the accompanying drawings, Figures 1 and 2 show the relationship between the number of nodules or spherules of graphite per mm.<sup>2</sup> and the nuclear formation temperature for periods of maintenance of this temperature of 48 and 96 hours respectively. Figure 3 shows the relationship between the number of nodules of graphite per mm.<sup>2</sup> and the period of maintaining various nuclear formation temperatures. The curves relate to the same malleable casting with the composition C=2.22%; Si=1.34%; Mn=0.65%; Cu=2%; S=0.12%; P=0.10%; Al=0.03%; Ti=0.06%. The advantage of

|                                                                                                               | Fe <sub>3</sub> C, Percent |                |                 |              | N            |                |                 |              |
|---------------------------------------------------------------------------------------------------------------|----------------------------|----------------|-----------------|--------------|--------------|----------------|-----------------|--------------|
|                                                                                                               | 1995 control               | 2145-I control | 2145-II Ni=1.83 | 2041 Cu=2.00 | 1995 control | 2145-I control | 2145-II Ni=1.83 | 2041 Cu=2.00 |
| Number of casting type of composition                                                                         |                            |                |                 |              |              |                |                 |              |
| Hardening, 450° C.; Kept 48 hours at 450° C.; Reheating 895° C., 14 hours                                     | 12                         |                | 5               | <1           | 0            |                | 60              | 250          |
| Preliminary hardening, 400° C.; 3 hours Nuclear formation 450° C.; 48 hours Graphitisation, 895° C., 14 hours |                            | 6              | 4               | 0            | 25           |                | 50              | 400          |

It will be seen that copper is more effective than nickel and that the latter treatment is better than the former. The increase in the number of nuclei given an equal addition is 3.8 times greater for copper than for nickel with the first treatment and 12.3 times greater with the second treatment. Compared on a basis of the same cost of addition, the copper would be 60 times more effective than nickel.

It is believed that this action of copper can be explained by the fact that it is in the neighbourhood of the ternary eutectic content Fe<sub>3</sub>C—Fe<sub>3</sub>C—Cu, so that it participates completely in the preliminary hardening while remaining in supersaturation in the ferrite. In the course of the nuclear formation treatment at 450° C., it undergoes a centripetal migration which precedes its precipitation. This leads to very high local increases in the copper concentration so that in these regions the instability of the cementite is increased and it decomposes,

60 observing a period sufficient to have a large number of nuclei of graphite and the economic disadvantage of prolonging this time excessively will be seen. Although the most satisfactory result is obtained at the end of 192 hours at 450° C., a period of 48 hours gives an almost identical result at a lower cost. On the other hand periods less than 30 hours sacrifice quality to no purpose.

With these castings containing 2% copper and cast in sand, and with correct treatment, the number of nodules or spherules of graphite per mm.<sup>2</sup> is generally between 3,000 and 15,000 according to the region and thickness, the average diameter of the spherules of graphite generally being between 1 and 10 microns, usually 4 microns.

The malleable castings containing copper, of the type forming the object of the invention, and the new precise series of heat treatment, have another remarkable new property in that they can extend the use of white iron

castings which can be rendered malleable to greater thicknesses of casting than by the conventional methods while combining white structure at the time of casting with suitability for graphitisation, which are generally contradictory properties. According to the invention, these properties are reconciled by the fact that on solidification, the graphitising action of 2% copper is compensated for by the whitening action of a corresponding increase in the manganese or by the introduction of molybdenum, or chromium, or the correlative reduction in silicon, whereas when the nuclei of graphite are formed at 450° C., this compensation no longer takes place, by reason of the centripetal migration of the copper which precedes its precipitation and the very high local increases in concentration which result therefrom.

A remarkable consequence of these new properties is the possibility of obtaining, by cupola smelting, by refining in a reverberatory furnace and by sandcasting, mouldings with a white structure which, after having been subjected to the triple treatment of preliminary hardening, nuclear formation, tempering and primary graphitisation annealing, have remarkable mechanical characteristics never before obtained in the industrial casting of white iron castings which can be rendered malleable, and this with a great regularity of production resulting both from the effect of the copper and from the precision in the heat treatment, without any risk of shrinkage cracks, due to the interrupted hardening, and without deforma-

10  
15

and tempering at 650° C., the elastic limit can be raised to give:

|                                        |     |
|----------------------------------------|-----|
| Vickers hardness, kg./mm. <sup>2</sup> | 350 |
| Elastic limit, kg./mm. <sup>2</sup>    | 98  |
| Breaking load, kg./mm. <sup>2</sup>    | 102 |
| Elongation, percent                    | 2.4 |

It is also possible to take advantage of the heat and the graphitisation annealing temperature to bring about the final treatment either by isothermal transformation or by hardening and tempering.

10  
15  
15

The favourable effect of copper as an additional constituent of cast irons in the three-phase treatment persists if the castings which are subjected thereto have been produced in metal chill-moulds. The effect of the copper is shown by the example quoted below in which are compared two chilled castings, the contents of which are identical apart from the copper and iron, namely:

| C, Percent | Si, Percent | Mn, Percent | S, Percent | P, Percent |
|------------|-------------|-------------|------------|------------|
| 2.40       | 1.55        | 0.60        | 0.10       | 0.10       |

20  
25  
25

The conditions of treating each of the two castings after preliminary hardening and the results obtained—number of nodules of graphite formed in the nuclear formation, and mechanical properties—are shown below:

| Copper introduced into the iron | Nuclear formation time and temperature | Number of nuclei per mm. <sup>2</sup> | Graphitisation time and temperature | Elastic limit, kg./mm. <sup>2</sup> | Breaking load, kg./mm. <sup>2</sup> | Elongation, percent |
|---------------------------------|----------------------------------------|---------------------------------------|-------------------------------------|-------------------------------------|-------------------------------------|---------------------|
| Nil                             | 15 hours at 500°                       | 18,000                                | 2 hours at 875°                     | 60                                  | 85                                  | 4                   |
| 1.20%                           | 15 hours at 450°                       | 38,000                                | 1 hour at 875°                      | 67                                  | 105                                 | 6.1                 |

tion because of the limitation of the highest temperature reached in the course of treatment.

The favourable effect of copper can be combined with that of additions of aluminum, titanium and zirconium, these three constituents having an equally favourable action for obtaining a large number of nuclei when the rational procedure of graphitisation with controlled nuclear formation is used. The following example relates to three castings of white iron cast in sand and having been subjected to the following treatment:

Heating to 810° C. for 30 minutes, quenching in salt at 180° C. for 1 minute, cooling in still air;

Reheating to 450° C. and maintaining for 48 hours, cooling in still air;

Reheating to 895° C. and maintaining for 14 hours, cooling in still air.

The following table gives the residual primary cementite and the number of nodules of graphite:

| Castings | C    | Si   | Mn   | S    | P    | Cu | Al   | Ti   | Zr    | Fe <sub>3</sub> C | N/mm. <sup>2</sup> |
|----------|------|------|------|------|------|----|------|------|-------|-------------------|--------------------|
| 2.203    | 2.49 | 1.19 | 0.65 | 0.07 | 0.08 | 0  | 0    | 0    | ----- | 1.5               | 1,200              |
| 2.205    | 2.53 | 1.25 | 0.61 | 0.07 | 0.08 | 2  | 0    | 0    | ----- | 0                 | 6,500              |
| 2.206    | 2.41 | 1.20 | 0.70 | 0.70 | 0.07 | 2  | 0.05 | 0.10 | ----- | 0                 | 6,500              |
| 2.207    | 2.41 | 1.20 | 0.07 | 0.07 | 0.07 | 2  | 0.03 | 0    | 0.12  | -----             | 8,000              |

65

The mechanical properties which can easily be obtained with these castings are generally at least equal to the following values for the test-pieces machined into bars and cooled in still air after graphitisation for 14 hours at 895° C., so that the matrix is lamellar pearlite:

|                                        |     |
|----------------------------------------|-----|
| Vickers hardness, kg./mm. <sup>2</sup> | 320 |
| Elastic limit, kg./mm. <sup>2</sup>    | 67  |
| Breaking load, kg./mm. <sup>2</sup>    | 82  |
| Elongation, percent                    | 4   |

70

But after the triple graphitisation treatment, these castings may also be subjected to a hardening and tempering process; thus by heating to 825° C., oil-hardening

5  
50  
50

ple 3 to 6 hours' maintenance at the temperature may be suitable.

White iron castings according to this process may also be produced in moulds the impression of which is constituted by relatively thin parts obtained by the agglomeration of sand or other refractory material, for example, by means of an organic thermosetting plastic material.

I claim:

1. A method of treating cast iron which comprises casting said iron in the form of a white iron casting having a thickness up to about 30 mm. and containing copper in a concentration of 0.7% to 3%, subjecting the casting of said white cast iron thus obtained to hardening by aus-

tenitization with heat at a temperature above the temperature at the end of the eutectoid transformation, followed by step quenching, to a temperature below the  $M_s$  whereby to form martensite, tempering at a temperature between 400 and 500° C. for 24 to 100 hours to effect the formation of nuclei in the graphite, and subjecting the casting to graphitization of the primary cementite by maintaining the casting at a temperature of about 875° C. to 900° C. for a period of time sufficient for the total disappearance of the cementite.

2. A method of treating cast iron which comprises casting said iron in the form of a white iron casting having a thickness up to about 30 mm. and containing copper in a concentration of 0.7% to 3%, subjecting the casting of said white cast iron thus obtained to hardening by austenitization with heat at a temperature above the temperature at the end of the eutectoid transformation, followed by step quenching including homogenization at a temperature slightly greater than the temperature at which martensitic transformation begins, followed by cooling in still air, tempering at a temperature between 400 and 500° C. for 24 to 100 hours to effect the formation of nuclei in the graphite, and subjecting the casting to graphitization of the primary cementite by maintaining the casting at a temperature of about 875° C. to 900 C. for a period of time sufficient for the total disappearance of the cementite.

3. A method of treating cast iron which comprises casting said iron in the form of a white iron casting having a thickness up to about 30 mm. and containing copper in a concentration of 0.7% to 3%, subjecting the casting of said white cast iron thus obtained to hardening by austenitization with heat at a temperature above the temperature at the end of the eutectoid transformation, followed by step quenching at the nuclear formation temperature to form martensite, tempering at a temperature between 400 and 500° C. for 24 to 100 hours to effect the formation of nuclei in the graphite, and subjecting the casting to graphitization of the primary cementite by maintaining the casting at a temperature of about 875° C. to 900° C. for a period of time sufficient for the total disappearance of the cementite.

4. A method of treating cast iron which comprises casting said iron in the form of a white iron casting having a thickness up to about 30 mm. and containing copper in a concentration of 0.7% to 3%, subjecting the casting of said white cast iron thus obtained to hardening by austenitization with heat at a temperature above the temperature at the end of the eutectoid transformation, followed by step quenching including homogenization at a temperature slightly greater than the temperature at which martensitic transformation begins, followed by cooling in still air, tempering at a temperature of about 450° C. for 36 to 48 hours to effect the formation of nuclei in the graphite, and subjecting the casting to graphitization of the primary cementite by maintaining the casting at a temperature of about 875° C. to 900° C. for a period of time sufficient for the total disappearance of the cementite and cooling in still air.

5. A method of treating cast iron which comprises casting said iron in the form of a white iron casting having a thickness up to about 30 mm. and containing copper in a concentration of 0.7% to 3% in a metal chill mold, subjecting the casting of said white cast iron thus obtained to hardening by austenitization with heat at a tempera-

ture above the temperature at the end of the eutectoid transformation, followed by step quenching to a temperature below the  $M_s$  whereby to form martensite, tempering at a temperature between 400 and 500° C. for 1 to 24 hours to effect the formation of nuclei in the graphite, and subjecting the casting to graphitization of the primary cementite by maintaining the casting at a temperature of about 875° C. to 900° C. for a period of time sufficient for the total disappearance of the cementite.

10. 6. A method of treating cast iron which comprises casting said iron in the form of a white iron casting having a thickness up to about 30 mm. and containing copper in a concentration of 0.7% to 3% in a metal chill mold, subjecting the casting of said white cast iron thus obtained to hardening by austenitization with heat at a temperature above the temperature at the end of the eutectoid transformation, followed by step quenching, to a temperature below the  $M_s$  whereby to form martensite, tempering at a temperature between 400 and 500° C. for 1 to 24 hours to effect the formation of nuclei in the graphite, and subjecting the casting to graphitization of the primary cementite by maintaining the casting at a temperature of about 875° C. to 895° C. for one-half to 2 hours.

7. A method as defined in claim 1, wherein the copper concentration is about 2%.

8. A method of treating cast iron which comprises casting said iron in the form of a white iron casting having a thickness up to about 30 mm. and containing copper in a concentration of 0.7% to 3%, subjecting the casting of said white cast iron thus obtained to hardening by austenitization with heat at a temperature above the temperature at the end of the eutectoid transformation, followed by step quenching, to a temperature below the  $M_s$  whereby to form martensite, tempering at a temperature between 400 and 500° C. for 1 to 24 hours to effect the formation of nuclei in the graphite, and subjecting the casting to graphitization of the primary cementite by maintaining the casting at a temperature of about 875° C. to 895° C. for one-half to 2 hours.

30. 9. A method of treating cast iron which comprises casting said iron in the form of a white iron casting having a thickness up to about 30 mm. and containing copper in a concentration of 0.7% to 3%, subjecting the casting of said white cast iron thus obtained to hardening by austenitization with heat at a temperature above the temperature at the end of the eutectoid transformation, followed by step quenching, to a temperature below the  $M_s$  whereby to form martensite, tempering at a temperature between 400 and 500° C. for 24 to 100 hours to effect the formation of nuclei in the graphite, and subjecting the casting to graphitization of the primary cementite by maintaining the casting at a temperature of about 875° C. to 895° C. for 10 to 14 hours.

40. 9. A method of treating cast iron which comprises casting said iron in the form of a white iron casting having a thickness up to about 300 mm. and containing copper in a concentration of 0.7% to 3%, subjecting the casting of said white cast iron thus obtained to hardening by austenitization with heat at a temperature above the temperature at the end of the eutectoid transformation, followed by step quenching, to a temperature below the  $M_s$  whereby to form martensite, tempering at a temperature between 400 and 500° C. for 24 to 100 hours to effect the formation of nuclei in the graphite, and subjecting the casting to graphitization of the primary cementite by maintaining the casting at a temperature of about 900° C. for 3 hours.

#### References Cited in the file of this patent

#### UNITED STATES PATENTS

|           |           |               |
|-----------|-----------|---------------|
| 1,489,128 | Sowers    | June 17, 1924 |
| 2,185,894 | Hultgren  | Jan. 2, 1940  |
| 2,331,886 | Boegehold | Oct. 19, 1943 |

#### OTHER REFERENCES

"Transactions of the American Foundrymen's Association," vol. 50, 1942, pages 1032, 1033.

"Material and Methods," vol. No. 32, Issue No. 6, December 1950, pages 50-53.